# EUROPEAN PATENT SPECIFICATION

(11) **EP 0 360 503 B1**
(45) Date of publication and mention of the grant of the patent: **19.05.1993**
(21) Application number: 89309379.9
(22) Date of filing: 15.09.1989
(51) Int. Cl.: C10M 173/02

(54) **Use of aqueous compositions in the plastic processing of metals**
Verwendung von wässrigen Zusammensetzungen für die plastische Verformung von Metallen
Utilisation de compositions aqueuses pour la formation plastique de métaux

(30) Priority: 19.09.1988 IT 2199888
(43) Date of publication of application: 28.03.1990
(73) Proprietor: AUSIMONT S.r.l., I-20100 Milano (IT)
(72) Inventor: Lafratta, Pietro, I-20135 Milan (IT); Chittofrati, Alba, I-20133 Milan (IT)
(74) Representative: Jones, Helen Marjorie Meredith

(56) References cited:
- EP-A- 0 250 766
- J. AM. CHEM. SOC., vol. 107, no. 5, 1985, pages 1197-2101; D.F. PERSICO et al.: "Synthesis of perfluoropolyethers via hydrocarbon polysters: A new general method"

## Description

The present invention relates to a liquid water-based composition useful as a lubricating and refrigerating liquid in the plastic processing of metals, which comprises, as a basic ingredient, a perfluoropolyethereal compound. The composition according to the invention is suitable in particular for rolling, dishing, drawing, pressing of metals in general, of ferrous and non-ferrous types such as steel, copper, aluminium and alloys thereof.

The use of liquids acting as lubricants in metal processing processes is well known. Such liquids, which generally consist of hydrocarbon oils with various additives for improving the performances thereof under severe operative conditions (high pressures, high temperatures), exhibit the drawback of being inflammable.

Recently, the use of aqueous emulsion with components having lubricating properties has been suggested. Such products are practically unaffected by the drawback of being inflammable under the operating conditions, and also satisfactorily fulfil the task of cooling the materials being processed. Lubricating compositions of this type are described for example in EP-A-0,048,216 (Alusuisse) CA-A-987,655 (Exxon), US-A-4,585,565 (Alcoa) and US-A-4,618,441 (Alcoa). Although many compositions in the form of aqueous emulsions have been suggested, it has been found that it is very difficult to prepare a composition which exhibits excellent performances as regards lubrication and cooling, a low friction coefficient (in order to achieve high reduction ratios) and which, furthermore, is endowed with good lubricating properties at high pressures and at the same time is free from various drawbacks such as instability of the emulsion which can lead to separation under the operating conditions.

A micro-emulsion is described in EP-A-250766. One suggested use of the micro-emulsion is in preparation of oil-based lubricants in order to ensure that water-soluble additives can be included.

The known compositions always require specific additives depending on the fields of use, in order to attain good values for the specific properties which are of major interest for the expected use.

The present invention comprises use of an aqueous composition comprising a perfluoropolyethereal compound having an average molecular weight of at least 400 with end groups of the perfluoropolyethereal chain consisting of perfluoroalkyls and/or of functional groups characterised in that the composition comprises from 1 to 40% by weight of the perfluoro - polyethereal compound at least 60% by weight water and the use is for a lubricating/refrigerating liquid in the cold plastic processing of metals.

The composition used according to the invention, besides exerting an excellent lubricating action, which allows a large reduction of thickness in a single run or pass in the rolling process, also effect an efficacious cooling of the material being processed by virtue of the high water content of the composition. The water content is at least 60% by weight and is preferably at least 80% by weight.

Furthermore, the compositions do not leave harmful product residues on the processed material, in a few cases it being possible to avoid a subsequent washing or rinsing. The compositions used according to the invention possess a high chemical stability and, if they are in the form of microemulsions, an unlimited physical stability. In addition, the residues remaining after evaporation of the water are non-inflammable.

An essential component of the lubricating-refrigerating compositions used according to the invention is a perfluoropolyether (PFPE) having an average molecular weight of at least 400 and preferably not higher than 5,000, with end groups of the perfluoropolyethereal chain of neutral type (perfluoroalkyl groups) and/or of polar functional type. The perfluoropolyethereal compound may be present in the aqueous composition either in the form of solution when the average molecular weight does not exceed 1,000 and the end groups are particularly hydrophilic(carboxylic groups), or in the form of microemulsions when the molecular weight exceeds 1,000 or alternatively when the average molecular weight is low and the end groups are neutral (perfluoroalkyl groups). The term "microemulsion" designates a liquid, macroscopically single-phase composition, which is limpid (transparent) or slightly opalescent (translucent), optically isotropic, indefinitely stable in a defined temperature range comprising the temperature at which said composition is used.

The microemulsions of both neutral and functional perfluoropolyether are prepared according to the ealier patent application EP-A-0,250,766.

Perfluoropolyethereal compounds which are particularly suitable as basic components of the aqueous composition used according to the present invention are the ones having a carboxylic end group suitably salified with organic or inorganic bases, in particular with ammonia or triethanolamine.

The amount of total perfluoropolyethereal compounds in the lubricating composition used according to the invention ranges from 1% to 40% by weight, preferably from 2% to 20%.

The perfluoropolyethers suited to form the lubricating compositions which are used according to the object of the present invention are in particular the ones which have an average molecular weight from 400 to 5,000 and preferably from 600 to 2,000, and belong in particular to one or more of the following classes:
1) with a random distribution of the perfluorooxyalkylene units, wherein R_{f} and R'_{f}, like or different from each other, are -CF₃-, -C₂F₅, -C₃F₇, or -COOH, -CF₂COOH, and m, n, p have such values as to meet the aforesaid average molecular weight requirements;
2) R_{f}O(CF₂CF₂O)ₙ(CF₂O)ₘR'_{f}, with a random distribution of the perfluorooxyalkylene units, wherein R_{f} and R'_{f}, like or different from each other, are -CF₃ or -C₂F₅, or -COOH, -CF₂COOH and m and n have such values as to meet the abovesaid requirements;
3) with a random distribution of the perfluorooxyalkylene units,wherein R_{f} and R'_{f} like or different from each other, are -CF₃, -C₂F₅ or -C₃F₇, or one of the above-indicated carboxylic radicals, and m, n, p, q have such values as to meet the abovesaid requirements;
4)
wherein R_{f} or R'_{f}, like or different from each other, are -C₂F₅ or -C₃F₇ or one of the above-indicated carboxylic radicals, and n has such a value as to meet the abovesaid requirements;
5) R_{f}O(CF₂CF₂O)ₙR'_{f} wherein R_{f} and R'_{f}, like or different from each other, are -CF₃, -C₂F₅, or one of the above-indicated carboxylic radicals, and n has such a value as to meet the abovesaid requirements;
6) R_{f}O(CX₂CF₂CF₂O)ₙR'_{f} wherein R_{f} and R'_{f}, like or different from each other, are -CF₃ or -C₂F₅ or -C₃F₇ or one of the above-indicated carboxylic radicals, X is F or H, n having such a value as to meet the abovesaid requirements;
7) wherein X is F or CF₃, R is F or Cl or Br or I, R', like or different from R, is also F or Cl or Br or I,
   Y is a -COOH group or a perfluoroalkyl group,
   T is a perfluoroalkyl group containing one or two atoms of Cl or Br or I; in particular it may be Alog CF₂-, Alog CF₂CF- where Alog is Cl or Br or I, CF₃
   n ranges from 1 to 15, the m/n ratio ranging from 0.01 to 0.5.

Perfluoropolyethers of class 1) are commercially available under the trademarks Fomblin^{R}Y or Galden^{R} and those of class 2) are commercially available under the trademark Fomblin^{R}Z, all being produced by Montedison.

Products of class 4), which are available on the market are the Krytox^{R}(du Pont). Products of class 5) are described in US-A-4,523,039 or in J. Am. Chem. Soc. 1985, 107, 1197-1201.

Products of class 6) are described in EP-A-0,148,482 in the name of Daikin.

The products of class 3) are prepared according to US-A-3,665,041.

The products of class 7) are described in European patent application Nos. 340740A and 340739A, both filed 2 May 1989 and published 8 November 1989 and in the name of the present applicant.

A second inessential but still very useful ingredient, in particular in order to increase the stability of the aqueous microemulsion when it contains non functional (neutral) PFPE, is a hydrogenated aliphatic alcohol, in particular isopropanol, or a fluorinated alcohol such as perfluoropolyether with end group -OH and a low molecular weight (≦ 450).

The alcohol amount in the aqueous composition may be as much as 20% by weight, but usually it does not exceed 10%. Useful compositions are described in previously cited EP-A-0,250,766.

The lubricating composition used according to the invention may furthermore contain small amounts of conventional additives such as components endowed with anticorrosive or antiwear properties, surfactants, EP additives, etc depending on the specific use they are intended for.

The formulations of a few lubricating compositions used according to the invention are indicated in the following examples, which are given for merely illustrative purposes. In Example 13 (Rolling and PSCT tests), alloys and mechanical characteristic thereof are disclosed eg in "Registration records of International alloy designation. Chemical Composition Limits for wrought aluminium and wrought alloy". Aluminium Association - Dusseldorf, Washington.

### Example 1

### Composition:

23.0 g of a monocarboxylic acid with perfluoropolyethereal structure belonging to class 1, having an average equivlent weight equal to 668,
- 7.8 ml of an ammonia aqueous solution at 10% by weight of ammonia;
- 53 ml of isopropyl alcohol;
- 384 ml of bidistilled water.

The sample contained 4.6% by weight of fluorinated substances and had a viscosity equal to 1.16 x 10⁻⁶m²/s (1.16 cst) at 40°C and an almost neutral pH (product reference: LR.1).

### Example 2

Composition:
- 9.4 g of ammonium salt of the monocarboxylic acid with perfluoropolyethereal structure belonging to class 1, having an average equivalent weight equal to 636;
- 1.3 g of a monofunctional alcohol having perfluoropolyethereal structure belonging to class 1, having an average equivalent weight equal to 600;
- 0.2 g of triethanolamine sebacate dissolved in 4.2 g of normal-butyl alcohol;
- 2.7 g of the PFPE having perfluoropolyethereal end groups belonging to class 1 and having an average molecular weight equal to 650 ;
- 82.2 g of bidistilled water.

The resulting O/W microemulsion contained 13.5% by weight of fluorinated substances and contained 0.2% of triethanolamine sebacate (product reference: 6/87).

### Example 3

Composition:
- 17.17 g of a monocarboxylic acid with perfluoropolyethereal structure belonging to class 1, having an average equivalent weight equal to 441;
- 8.8 ml of an ammonia aqueous solution at 10% by weight of NH₃;
- 284 ml of bidistilled water.

The solution contained 5.05% by weight of fluorinated substances and had a viscosity of 0.75 x 10⁻⁶m²/s (0.75 cst) at 40°C; the pH was equal to 8.2 (product reference: LR.3).

### Example 4

Composition:
- 150.4 g of a monocarboxylic acid with perfluoropolyethereal structure belonging to class 1, having an average equivalent weight equal to 443 and a narrow molecular weight distribution;
- 52.1 g of an ammonia solution at 10% by weight of ammonia;
- 10.8 g of a perfluoropolyether having an average molecular weight equal to about 1,200;
- 32.4 g of a fluorinated alcohol having a perfluoropolyethereal structure and a molecular weight equal to 678;
- 23.0 g of isopropyl alcohol;
- 293.1 ml of bidistilled water.

The resulting microemulsion contained 6.5% by weight of fluorinated substances and had a pH equal to 4.4 (product reference: LR.17).

### Example 5

Composition:
- 18.39 g of a monocarboxylic acid having perfluoropolyethereal structure belonging to class 7, having a chlorofluoroalkyl end group for each molecule and having an average equivalent weight of about 850 and a wide distribution of the molecular weights;
- 6.44 g of an aqueous ammonia solution at 10% by weight of NH₃;
- 338 g of bidistilled water.

The obtained solution contained 5.1% by weight of chlorofluorinated substances and had a pH equal to 8.3 (product reference: LR.15).

### Example 6

Composition:
- 19.8 g of a perfluoropolyether belonging to class 1 having carboxylic end groups and an average molecular weight equal to 4170;
- 14.6 g of isopropyl alcohol;
- 2.2 g of monocarboxylic acid having perfluoropolyethereal structure, belonging to class 1, having an average equivalent weight of 668;
- 63.4 g of aqueous phase containing the ammonia which is necessary to salify the carboxylic groups.

The O/W microemulsion obtained by mixing the above-listed components was a fluid, clear between 25° and 75°C, containing a viscosity of 3.8 x 10⁻⁵m²/s (38 cst) at 40°C (product reference: LR.A).

### Example 7

Composition:
- 5.3 g of a functionalized perfluoropolyether belonging to class 1, having carboxylic end groups and an average molecular weight equal to 2080;
- 19.2 g of isopropyl alcohol;
- 75.5 g of an aqueous solution containing the ammonia which is necessary to salify the carboxylic groups.

The O/W microemulsion obtained by mixing the abovesaid components was a fluid, limpid between 25° and 50°C, containing 5.3% by weight of fluorinated substances and having a viscosity of 2.25 x 10⁻⁶m²/s (2.25 cst) at 40°C (product reference: LR.C).

### Example 8

Composition:
- 25.2 g of a monocarboxylic acid having perfluoropolyethereal structure, belonging to class 1, having an average equivalent weight equal to 668 and a wide distribution of the molecular weights;
- 9.1 ml of an aqueous ammonia solution at 10% by weight of ammonia;
- 1.4 ml of a perfluoropolyether having perfluoroalkyl end groups, belonging to class 1 and having an average molecular weight equal to 650;
- 28 ml of isopropanol;
- 280 ml of bidistilled water.

The sample was stable in the whole temperature range taken into examination contained 8.2% by weight of fluorinated substances and had a viscosity of 1.2 x 10⁻⁶m²/s (1.2 cst) at 40°C, the pH being equal to 8 (product reference: LR.5).

### Example 9

Composition:
- 55.0 g of a monocarboxylic acid having perfluoropolyethereal structure belonging to class 7, having a chlorofluoralkyl end group per molecule and having an average equivalent weight of about 478 and a wide molecular weight distribution;
- 62.14 g of triethanolamine;
- 10.14 g of bidistilled water.

The resulting solution contained 4.86% by weight of chlorofluorinated substances and had a pH equal to 8.36 (product reference: LR.15 TEA).

### Example 10

Composition:
- 26.18 g of ammonium salt of the acid belonging to class 1, having an average equivalent weight equal to 441;
- 1.4 g of a perfluoropolyether of class 1, having perfluoroalkyl end groups and an average molecular weight of about 650;
- 5.6 ml of isopropyl alcohol;
- 293 ml of bidistilled water.

The system was limpid in the whole temperature range. It contained 8.8% by weight of fluorinated substances and had a viscosity of 0.85 x 10⁻⁶m²/s (0.85 cst) at 40°C; it was brought to a pH = 8 by adding thereto 0.15 ml of an ammonia solution at 10% by weight of ammonia (product reference: LR.7).

### Example 11

Composition:
- 35.1 g of a monocarboxylic acid of perfluoropolyethereal structure belonging to class 1, having an average equivalent weight equal to 668 and a wide distribution of the molecular weights;
- 5.4 g of a monocarboxylic acid of perfluoropolyethereal structure belonging to class 1, having an average equivalent weight equal to 443 and a narrow distribution of the molecular weights;
- 11.3 g of ammonia solution at 10%;
- 2.8 g of a perfluoropolyether of class 1, having perfluoroalkyl end groups and an average molecular weight of about 1,200;
- 23.6 g of isopropyl alcohol;
- 300 ml of bidistilled water.

The microemulsion so obtained was stable in the whole temperature range. It contained 11.4% by weight of fluorinated substances and had a pH equal to 7.4. (Product reference: LR.9).

The following examples describe the preparation of additive-containing microemulsions.

### Example 12

Composition:
- 108.0 g of a monocarboxylic acid with perfluoropolyethereal structure belonging to class 1, having an average equivalent weight equal to 668;
- 1.8 g of a monocarboxylic acid with perfluoropolyethereal structure belonging to class 1, having an average equivalent weight equal to 443 and a narrow distribution of the molecular weights;
- 33.7 g of ammonia solution at 10%;
- 33.4 g of perfluoropolyether having an average molecular weight of about 1,200;
- 23.6 g of a solution of triethanolamine sebacate in isopropanol, at 10.2% by weight;
- 3.1 g of isopropanol;
- 240 ml of bidistilled water.

The resulting O/W microemulsion contained 32.3% by weight of fluorinated substances and 0.6% by weight of triethanolamine sebacate, and had a pH equal to 7.6 (product reference: LR.10).

### Example 13

90.3 g of the sample described in the preceding example 12 was diluted with 250 ml of water.
The resulting O/W microemulsion contained 8.6% by weight of fluorinated substances and 0.2% by weight of triethanolamine sebacate, the pH being equal to 5.3 (product reference: LR.11).

The utilization characteristics of the lubricating compositions according to the invention, with reference to specific applications, are illustrated in detailed hereinafter.

### Rolling

The lubricating compositions under examination were subjected to the "Plane Strain Compression Test" (paper 2015 by R.D. Guminski and J. Willis - Journal of the Institute of Metals, 1959-60, vol 88). The Plane Strain Compression Test is an improvement of the BISRA Compression Test (see The Rolling of Metals by L.R. Underwood, pages 116-119 - Chapman and Hall - London 1952) and is well indicative of the thickness reduction capacity of the lubricants in the cold-rolling of aluminium: the data determined in the plane strain compression test are well in correlation to the behaviour in use exhibited by the lubricating mixtures.
Further literature sources on the P.S.C.T., which extend the validity of the test also to steel, are : Kubie and Delamare - Journal of Lubrication Technology, pages 538-551 - 1982, vol. 104).
The test carried out according to Guminski/Willis was the following : A 50x2.52x150 mm strip of aluminium alloy 3003 - H22 was subjected, after wetting with the lubricant, to 5 successive compressions between two vertical plates measuring 75x6.20 mm in a press mounted in a traction/compression machine, the whole in accordance with the indication given by Guminski and Willis, with the exception that the applicated load was of 6,800 kg in order to make the test more selective.
The fluids of the present invention can be applicated to the metal surface according to conventional methods such as immersion, spraying, and by means of jets, brushes, wiping, rollers or the like.
In the following examples, the composition was applied by brush.
The results are reported in the following Table 1.

Determination of the friction coefficient by means of the Plane Strain Compression Test (PSCT), as is described by Kubie and Delamare in the above-cited literature. Also this test, which provides the friction coefficient values, permits to evaluate the reduction ratios obtainable in the rolling process.
Metal test-piece (20x300 mm sheet thickness: about 0.6 mm), applicated load: 10,000 kg:
a) steel at 0.03% of C and 1% of Mn, annealed;
b) Al/Mg alloy 5052 0, annealed.

The test-pieces were degreased by means of acetone before being tested.

### Tested lubricants:

a) composition of example 1 (LR.1);
b) composition of example 5 (LR. 15);
c) composition example 7 (LR.C) ;
d) composition of example 9 (LR. 15 TEA);
e) rolling oil for the steel referred to as Q.27, a commercial product having the following composition:
f) emulsion of preceding product Q.27 at 10% by weight of water;
g) palm oil;
h) product which is an aqueous emulsion at 4% by weight of the following oily composition:

The tests on steel were carried out with a load corresponding to a thickness reduction of about 30%; the tests on Al alloy were conducted at a pressure corresponding to a thickness reduction of about 60%.
The results are indicated in Tables 2 and 3.

### Dishing

Dishing is the process by means of which a metal plate is subjected to permanent plastic deformation by buckling between two surfaces (die and punch).

The lubricant must have good EP characteristics (high pressures), i.e. it must secure the sliding between two metal surfaces (sheet iron to be deformed and dies) under a high pressure, and that is achieved by lubricants which do not exhibit any film rupture under such conditions. In general different lubricants are utilized at present, depending on the type of dishing to be carried out and on the materials to be worked; the lubricants may be a mineral oil with various additives, as well as soap baths, emulsions, waxes, greases, fluoride and phosphate baths, chloroparaffins, polymeric resins, graphite or MoS₂ in oil etc.

The PFPE-based aqueous compositions according to the present invention are suited also as lubricants for the dishing process.

The use of these compositions in this type of application is novel. The compositions are suited to the dishing of metals as they permit a dishing ratio comparable to the ones obtainable with whole oils based on hydrocarbons, while remarkably reducing the necessity to degrease the sheets for the subsequent processing steps.

The compositions of the invention may further contain minor amounts of additives for particular operative conditions if necessary. Such additives may be for instance corrosion inhibitors, antistatic agents, surfactants or slippage agents.

### Examples

The fluids of the invention were subjected to the Erichsen test (UN 8341) on steel FE PO4, (UNI).

The fluids of the present invention are applicable to the metal surface by means of conventional methods such as dipping, spraying, wiping, by brushes, roller or the like. The results, which are reported on the following table 4, indicate the depth of penetration, in tenths of mm, of the punch into a sheet-steel having a roughness of 0.8 microns.

### Lubricating properties of the fluids according to the invention.

For the fluids utilized in several plastic processings of metals, good EP characteristics may be required.
In order to determine the EP characteristics of the microemulsions and aqueous solutions of perfluoropolyethers and derivatives thereof, "Shell 4 balls" tests (IP 239/79) were carried out.
The "Shell 4 balls" tests were always carried out using balls made of steel UNI 100 Cr₆.

### Examples

The fluids according to the invention were subjected to the "Shell 4 balls" test (IP 239/79 ASTM D2783).
The results are indicated in the following table.

## Claims

1. Use of an aqueous composition comprising a perfluoropolyethereal compound having an average molecular weight of at least 400 with end groups of the perfluoropolyethereal chain consisting of perfluoroalkyls and/or of functional groups characterised in that the composition comprises from 1 to 40% by weight of the perfluoro polyethereal compound, at least 60% by weight water and that the use is for a lubricating/refrigerating liquid in the cold plastic processing of metals.

2. Use according to claim 1 in which the processing includes rolling, dishing and/or drawing.

3. Use according to any preceding claim in which the perfluoropolyether has carboxylic end groups which are salified, preferably with ammonia or triethanolamine.

4. Use according to any preceding claim in which the composition is in the form of a microemulsion.

5. Use according to any preceding claim in which the the perfluoropolyether has an average molecular weight in the range from 400 to 5,000, preferably 600 to 2,000.

6. Use according to any preceding claim in which the perfluoropolyether is selected from the following classes:
1) with a random distribution of the perfluorooxyalkylene units, wherein R_{f} and R'_{f} like or different from each other, are -CF₃-, -C₂F₅, -C₃F₇, or -COOH, -CF₂COOH, and m, n, p have such values as to meet the aforesaid average molecular weight requirements;
2) R_{f}O(CF₂CF₂O)ₙ(CF₂O)ₘR'_{f}, with a random distribution of the perfluorooxyalkylene units, wherein R_{f} and R'_{f}, like or different from each other, are -CF₃ or -C₂F₅, or -COOH, -CF₂COOH and m and n have such values as to meet the abovesaid requirements;
3) with a random distribution of the perfluorooxyalkylene units,wherein R_{f} and R'_{f}, like or different from each other, are -CF₃, -C₂F₅ or -C₃F₇, or one of the above-indicated carboxylic radicals, and m, n, p, q have such values as to meet the abovesaid requirements;
4) wherein R_{f} or R'_{f}, like or different from each other, are -C₂F₅ or -C₃F₇ or one of the above-indicated carboxylic radicals, and n has such a value as to meet the abovesaid requirements;
5) R_{f}O(CF₂CF₂O)ₙR'_{f} wherein R_{f} and R'_{f}, like or different from each other, are -CF₃, -C₂F₅, or one of the above-indicated carboxylic radicals, and n has such a value as to meet the abovesaid requirements;
6) R_{f}O(CX₂CF₂CF₂O)ₙR'_{f} wherein R_{f} and R'_{f}, like or different from each other, are -CF₃ or -C₂F₅ or -C₃F₇ or one of the above-indicated carboxylic radicals, X is F or H, n having such a value as to meet the abovesaid requirements;
7) wherein X is F or CF₃, R is F or Cl or Br or I, R', like or different from R, is also F or Cl or Br or I,
Y is a -COOH group or a perfluoroalkyl group,
T is a perfluoroalkyl group containing one or two atoms of Cl or Br or I; in particular it may be Alog CF₂-, where Alog is Cl or Br or I,
n ranges from 1 to 15, the m/n ratio ranging from 0.01 to 0.5.

## Patentansprüche

1. Verwendung einer wäßrigen Zusammensetzung, umfassend eine Perfluorpolyether-Verbindung mit einem durchschnittlichen Molekulargewicht von mindestens 400 mit Endgruppen der Perfluorpolyetherkette, bestehend aus Perfluoralkylgruppen und/oder funktionellen Gruppen, dadurch gekennzeichnet, daß die Zusammensetzung 1 bis 40 Gewichtsprozent Perfluorpolyether-Verbindung und mindestens 60 Gewichtsprozent Wasser umfallt und daß die Verwendung für eine Schmier-/Kühlflüssigkeit bei der plastischen Kaltbearbeitung von Metallen ist.

2. Verwendung nach Anspruch 1, worin die Bearbeitung das Walzen, Tiefziehen und/oder Ziehen einschließt.

3. Verwendung nach irgendeinem vorangehenden Anspruch, worin der Perfluorpolyether Carboxyl-Endgruppen umfaßt, die in ein Salz überführt sind, vorzugsweise mit Ammoniak oder Triethanolamin.

4. Verwendung nach irgendeinem vorangehenden Anspruch, worin die Zusammensetzung in Form einer Mikroemulsion vorliegt.

5. Verwendung nach irgendeinem vorangehenden Anspruch, worin der Perfluorpolyether ein durchschnittliches Molekulargewicht im Bereich von 400 bis 5000, vorzugsweise 600 bis 2000 hat.

6. Verwendung nach irgendeinem vorangehenden Anspruch, worin der Perfluorpolyether aus den folgenden Klassen ausgewählt ist:
1) mit einer statistischen Verteilung der Perfluoroxyalkylen-Einheiten, worin R_{f} und R'_{f} gleich oder verschieden voneinander -CF₃, -C₂F₅, -C₃F₇ oder -COOH, -CF₂COOH sind und m, n, p solche Werte haben, daß die oben genannten Anforderungen hinsichtlich des durchschnittlichen Molekulargewichts erfüllt sind;
2) R_{f}O(CF₂CF₂O)ₙ(CF₂O)ₘR'_{f}, mit einer statitischen Verteilung der Perfluoroxyalkylen-Einheiten, worin R_{f} und R'_{f} gleich oder verschieden voneinander sind und -CF₃ oder -C₂F₅ oder -COOH, -CF₂COOH sind und m und n solche Werte haben, daß die oben genannten Anforderungen erfüllt sind;
3) mit einer statistischen Verteilung der Perfluoroxyalkylen-Einheiten, worin R_{f} und R'_{f} gleich oder verschieden voneinander -CF₃, -C₂F₅ oder -C₃F₇ oder einer der oben genannten Carboxylreste sind und m, n, p, q solche Werte haben, daß die oben genannten Anforderungen erfüllt sind;
4) worin R_{f} oder R'_{f} gleich oder verschieden voneinander -C₂F₅ oder -C₃F₇ oder einer der oben genannten Carboxylreste sind und n einen solchen Wert hat, daß die oben genannten Anforderungen erfüllt sind;
5) R_{f}O(CF₂CF₂O)ₙR'_{f}, worin R_{f} oder R'_{f} gleich oder verschieden voneinander -CF₃, -C₂F₅ oder einer der oben genannten Carboxylreste sind und n einen solchen Wert hat, daß die oben genannten Anforderungen erfüllt sind;
6) R_{f}O(CX₂CF₂CF₂O)ₙR'_{f}, worin R_{f} oder R'_{f} gleich oder verschieden voneinander -CF₃ oder -C₂F₅ oder -C₃F₇ oder einer der oben genannten Carboxylreste sind, X F oder H ist, n einen solchen Wert hat, daß die oben genannten Anforderungen erfüllt sind;
7) worin X F oder CF₃ ist, R F oder Cl oder Br oder I ist, R' gleich oder verschieden von R ebenfalls F oder Cl oder Br oder I ist, Y eine -COOH Gruppe oder Perfluoralkylgruppe ist, T eine Perfluoralkylgruppe ist, die ein oder mehrere Atome von Cl oder Br oder I enthält; insbesondere kann es Alog CF₂-, sein, worin Alog Cl oder Br oder I ist, n im Bereich von 1 bis 15 liegt, wobei das Verhältnis m/n im Bereich von 0,01 bis 0,5 liegt.

## Revendications

1. Utilisation d'une composition aqueuse compre-nant un composé perfluoropolyéthéré ayant un poids moléculaire moyen d'au moins 400 avec des groupes terminaux de la chaîne perfluoropolyéthérée consistant en groupes perfluoroalkyles et/ou groupes fonctionnels, caractérisée en ce que la composition comprend de 1 à 40% en poids du composé perfluoropolyéthéré, au moins 60% en poids d'eau et qu'elle convient pour un emploi en tant que liquide de lubrification/réfrigération pour le formage classique à froid des métaux.

2. Utilisation suivant la revendication 1 dans laquelle le formage comprend le laminage, l'emboutissage et/ou l'étirage.

3. Utilisation suivant l'une quelconque des revendications précédentes dans laquelle le perfluoropolyéther a des groupes terminaux carboxyliques qui sont salifiés, de préférence avec de l'ammoniac ou de la triéthanolamine.

4. Utilisation suivant l'une quelconque des revendications précédentes dans laquelle la composition est sous la forme d'une micro-émulsion.

5. Utilisation suivant l'une quelconque des revendications précédentes dans laquelle le perfluoropolyéther a un poids moléculaire moyen de l'ordre de 400 à 5000, de préférence de 600 à 2000.

6. Utilisation suivant l'une quelconque des revendications précédentes dans laquelle le perfluoropolyéther est choisi dans les classes suivantes:
1) avec une distribution aléatoire des unités perfluorooxyalkylènes, R_{f} et R'_{f}, identiques ou différents l'un de l'autre étant les groupes -CF₃-, C₂F₅, -C₃F₇ ou -COOH, -CF₂COOH, et m, n, p ayant des valeurs convenables pour satisfaire aux conditions requises de poids moléculaire moyen indiqué plus haut;
2) R_{f}O(CF₂-CF₂O)ₙ(CF₂O)ₘR'_{f}
avec une distribution aléatoire des unités perfluoroxyalkylènes, R_{f} et R'_{f}, identiques ou différents l'un de l'autre, étant les groupes -CF₃ ou -C₂F₅, -COOH, -CF₂COOH, et m et n ayant des valeurs convenables pour satisfaire aux conditions requises mentionnées plus haut;
3) avec une distribution aléatoire des unités perfluorooxyalkylènes, R_{f} et R'_{f}, identiques ou différents l'un de l'autre, étant les groupes -CF₃-, C₂F₅ ou -C₃F₇ ou l'un des groupes carboxyliques indiqués plus haut, et m, n, p et q ayant des valeurs convenables pour satisfaire aux conditions requises mentionnées plus haut;
4) R_{f} et R'_{f}, identiques ou différents l'un de l'autre, étant des groupes -C₂F₅ ou -C₃F₇ ou l'un des radicaux carboxyliques indiqués plus haut et n ayant une valeur convenable pour satisfaire aux conditions requises mentionnées plus haut;
5) R_{f}O(CF₂CF₂O)ₙ-R'_{f}
R_{f} et R'_{f}, identiques ou différents l'un de l'autre, étant des groupes -CF₃, -C₂F₅ ou l'un des radicaux carboxyliques indiqués plus haut et n ayant une valeur convenable pour satisfaire aux conditions requises mentionnées plus haut;
6) R_{f}O(CX₂CF₂CF₂O)ₙ-R'_{f}
R_{f} et R'_{f}, identiques ou différents l'un de l'autre, étant des groupes -CF₃ ou -C₂F₅ ou -C₃F₇ ou l'un des radicaux carboxyliques indiqués plus haut, X est F ou H, n ayant une valeur convenable pour satisfaire aux conditions requises mentionnées plus haut;
7)
X étant F ou CF₃, R étant F, Cl, Br ou I, R', identiques ou différents de R étant également F, Cl, Br ou I,
Y étant un groupe -COOH ou un groupe perfluoroalkyle,
T étant un groupe perfluoroalkyle contenant un ou deux atomes de chlore, brome ou iode; en particulier T pouvant être un groupe Halog-CF₂-, où Halog est Cl, Br ou I,
n étant de l'ordre de 1 à 15, et tel que le rapport m/n soit compris entre 0,01 et 0,5.
